



US010754270B2

(12) **United States Patent**  
**Kitada et al.**

(10) **Patent No.:** **US 10,754,270 B2**  
(b5) **Date of Patent:** **Aug. 25, 2020**

(54) **TONER, PRODUCTION METHOD OF TONER, IMAGE FORMING METHOD, IMAGE FORMING APPARATUS, AND PROCESS CARTRIDGE**

(71) Applicants: **Naoko Kitada**, Shizuoka (JP); **Satoshi Ogawa**, Nara (JP); **Yoshitaka Sekiguchi**, Shizuoka (JP); **Masayuki Ishii**, Shizuoka (JP); **Shohta Kobayashi**, Shizuoka (JP)

(72) Inventors: **Naoko Kitada**, Shizuoka (JP); **Satoshi Ogawa**, Nara (JP); **Yoshitaka Sekiguchi**, Shizuoka (JP); **Masayuki Ishii**, Shizuoka (JP); **Shohta Kobayashi**, Shizuoka (JP)

(73) Assignee: **Ricoh Company, Ltd.**, Tokyo (JP)

(\*) Notice: Subject to any disclaimer, the term of this patent is extended or adjusted under 35 U.S.C. 154(b) by 0 days.

(21) Appl. No.: **16/492,818**

(22) PCT Filed: **Feb. 15, 2018**

(86) PCT No.: **PCT/JP2018/005299**

§ 371 (c)(1),  
(2) Date: **Sep. 10, 2019**

(87) PCT Pub. No.: **WO2018/168312**

PCT Pub. Date: **Sep. 20, 2018**

(65) **Prior Publication Data**

US 2020/0174390 A1 Jun. 4, 2020

(30) **Foreign Application Priority Data**

Mar. 17, 2017 (JP) ..... 2017-053250

(51) **Int. Cl.**

**G03G 9/08** (2006.01)  
**G03G 9/097** (2006.01)

(Continued)

(52) **U.S. Cl.**  
CPC ..... **G03G 9/09783** (2013.01); **G03G 9/081** (2013.01); **G03G 9/0815** (2013.01);  
(Continued)

(58) **Field of Classification Search**  
CPC ..... G03G 9/0815; G03G 9/0819  
(Continued)

(56) **References Cited**

U.S. PATENT DOCUMENTS

|                 |         |                 |
|-----------------|---------|-----------------|
| 5,714,294 A     | 2/1998  | Maruta et al.   |
| 2007/0275315 A1 | 11/2007 | Nagatomo et al. |

(Continued)

FOREIGN PATENT DOCUMENTS

|    |               |         |
|----|---------------|---------|
| EP | 0737899 A1    | 10/1996 |
| JP | 2006-139051 A | 6/2006  |
| JP | 2009-025749 A | 2/2009  |

OTHER PUBLICATIONS

International Search Report dated Apr. 24, 2018 for counterpart International Patent Application No. PCT/JP2018/005299 filed Feb. 15, 2018.

(Continued)

*Primary Examiner* — Mark A Chapman

(74) *Attorney, Agent, or Firm* — Oblon, McClelland, Maier & Neustadt, L.L.P.

(57) **ABSTRACT**

Provided is a toner including a binder resin, and a charge-controlling agent, wherein a volume average particle diameter X of the toner after a stress treatment satisfies Formula (1), and an amount Y of fine toner particles having particle diameters of 3 micrometers or smaller and circularity of 0.70 or less satisfies Formula (2).

**9 Claims, 3 Drawing Sheets**



- (51) **Int. Cl.**  
*G03G 9/087* (2006.01)  
*G03G 21/18* (2006.01)  
*G03G 15/08* (2006.01)
- (52) **U.S. Cl.**  
CPC ..... *G03G 9/0817* (2013.01); *G03G 9/0819* (2013.01); *G03G 9/08755* (2013.01); *G03G 15/08* (2013.01); *G03G 21/1803* (2013.01)
- (58) **Field of Classification Search**  
USPC ..... 430/110.1, 137.1  
See application file for complete search history.

(56) **References Cited**

U.S. PATENT DOCUMENTS

- 2008/0227009 A1 9/2008 Fuwa et al.  
2009/0029280 A1 1/2009 Yamamoto et al.  
2009/0068579 A1 3/2009 Ogawa et al.  
2009/0074467 A1 3/2009 Seshita et al.  
2009/0233218 A1 9/2009 Ogawa  
2010/0291481 A1 11/2010 Yamada et al.  
2013/0344433 A1 12/2013 Casalmir et al.  
2016/0327884 A1 11/2016 Nakajima et al.

OTHER PUBLICATIONS

Written Opinion dated Apr. 24, 2018 for counterpart International Patent Application No. PCT/JP2018/005299 filed Feb. 15, 2018.

[Fig. 1]



[Fig. 2]



[Fig. 3]



[Fig. 4]



[Fig. 5]



[Fig. 6]



**TONER, PRODUCTION METHOD OF  
TONER, IMAGE FORMING METHOD,  
IMAGE FORMING APPARATUS, AND  
PROCESS CARTRIDGE**

**TECHNICAL FIELD**

The present disclosure relates to a toner, a production method of the toner, an image forming method, an image forming apparatus, and a process cartridge.

**BACKGROUND ART**

One-component development is performed by pressing a supply roller etc. against a developing roller to supply a toner on the developing roller, making the toner to be electrostatically held on the developing roller, forming the toner into a thin layer with a regulating blade, friction-charging the toner, and supplying the toner to a photoconductor to develop with the toner. One-component development can realize downsize in weight and cost saving compared to two-component development or magnetic one-component development.

Moreover, sizes of particles of a toner obtained by pulverization have been reduced in order to improve image quality and therefore there is a need for homogeneously disperse a colorant, a charge-controlling agent, or a release agent in a thermoplastic resin. When dispersion is insufficient, the colorant, charge-controlling agent, or release agent added to the toner comes at an outer surface of the toner particle in the process of pulverization. As a result, irregular-shape toner particles having a low average circularity are generated in a very fine powder region having particle diameters of 3 micrometers or smaller. When toner particles are observed per single particle, moreover, there are problems, such as variations in amounts of raw materials contained in the toner particle, and an increase in an amount of the raw materials exposing to a surface of the toner particle. Accordingly, toner-charging failures occur due to unevenness of the toner particles, and problems, such as conveying failures and deterioration in image quality due to background smear, occur.

In order to solve the above-described problems, proposed are to regulate a ratio of toner particles having the low average circularity or an abundance ratio of toner particles having different circularity to a certain range, to control an abundance of very fine powder region (3 micrometers or smaller) to a certain value or lower, and to control shapes of toner particles in the very fine powder region.

For example, PTL 1 (Japanese Unexamined Patent Application Publication No.

2009-25749) discloses a toner for the purpose of providing a toner having excellent flowability and capable of forming a high quality image of high definition and high resolution, a production method of the toner, a two-component developer, a developing device, and an image forming apparatus. The toner includes at least a binder resin and a colorant. The toner includes a particle group of a large particle diameter and a particle group of a small particle diameter. A volume average particle diameter of the small particle diameter-particle group is smaller than a volume average particle diameter of the large particle diameter-particle group. A volume average particle diameter  $D_{50V}$  a cumulative volume of which from the large particle diameter side in a cumulative volume distribution is 50% is 4 micrometers or greater but 8 micrometers or smaller. An amount of toner particles having a volume average particle diameter of

7 micrometers or greater is 24% by volume or greater but 47% by volume or less. An amount of toner particles having a number average particle diameter of 5 micrometers or less is 10% by number or greater but 50% by number or less.

Moreover, PTL 2 (Japanese Unexamined Patent Application Publication No. 2006-139051) discloses a toner used for a two-component developer including a silicone-coated carrier and the toner for the purpose of providing an excellent electrostatic latent image-developing toner and two-component developer where a charge-controlling agent is securely fixed on surfaces of particles of the toner even when the low-fixing toner is used, fogging caused particularly by a difference in a charge amount between the toner in the developer and the supply toner is prevented, and deterioration of the developer is prevented. The toner includes toner base particles each including at least a binder resin, a colorant, and a release agent, a charge-controlling agent, and inorganic particles. When the toner is supplied, an average circularity of the toner measured by a flow particle image analyzer is 0.930 through 0.965 and an amount of fine particles of 3 micrometers or smaller is 5% by number through 20% by number. After the toner is supplied, an amount of fine particles of 3 micrometers or smaller in the toner in a developing device is 5% by number through 70% by number.

**CITATION LIST**

**Patent Literature**

[PTL 1] Japanese Unexamined Patent Application Publication No. 2009-25749

[PTL 2] Japanese Unexamined Patent Application Publication No. 2006-139051

**SUMMARY OF INVENTION**

**Technical Problem**

The present disclosure has an object to provide a toner which has excellent fixing ability (low-temperature fixing ability and hot offset resistance) and can prevent deterioration of image quality caused by background smear even after the toner receives stress.

**Solution to Problem**

According to one aspect of the present disclosure, a toner includes a binder resin and a charge-controlling agent. A volume average particle diameter  $X$  of the toner after a stress treatment below satisfies Formula (1) below. An amount  $Y$  of fine toner particles having particle diameters of 3 micrometers or smaller and circularity of 0.70 or less satisfies Formula (2) below.

$$6.0 \leq X(\text{micrometers}) \leq 8.5 \quad \text{Formula (1)}$$

$$Y(\%) \leq 4.3X(\text{micrometers}) - 14.6 \quad \text{Formula (2)}$$

The stress treatment includes charging a container formed of polypropylene having a volume of 100 mL with 5 g of the toner and 10 g of alumina beads having particle diameters of 0.5 mm, and shaking the toner by shaking the container using a shaker (YS-8D, available from YAYOI Co., Ltd.) with a stroke width of 80 mm, a stroke number of 250 times/min, and a shaking duration of 1 hour.

**Advantageous Effects of Invention**

The present disclosure can provide a toner which has excellent fixing ability (low-temperature fixing ability and

hot offset resistance) and can prevent deterioration of image quality caused by background smear even after the toner receives stress.

#### BRIEF DESCRIPTION OF DRAWINGS

FIG. 1 is a graph depicting a relationship between a volume average particle diameter X of a toner after a stress treatment and an amount Y of fine toner particles.

FIG. 2 is a view for describing one embodiment of a process cartridge of the present disclosure.

FIG. 3 is a view for describing one embodiment of an image forming apparatus of the present disclosure.

FIG. 4 is a view for describing another embodiment of the image forming apparatus of the present disclosure.

FIG. 5 is a view for describing another embodiment of the image forming apparatus of the present disclosure.

FIG. 6 is a view for describing an image forming unit.

#### DESCRIPTION OF EMBODIMENTS

It cannot be said that toners available in the art have yet sufficiently solved a problem associated with deterioration of image quality caused by background smear.

Moreover, there is no suggestion in the art for a problem of background smear or deterioration of image quality caused by a toner after receiving stress.

Accordingly, the present disclosure has an object to provide a toner which has excellent fixing ability (low-temperature fixing ability and hot offset resistance) and can prevent deterioration of image quality caused by background smear even after the toner receives stress.

Embodiments of a toner of the present disclosure, a production method of the toner, an image forming method, an image forming apparatus, and a process cartridge will be more specifically described hereinafter.

A toner of the present disclosure includes a binder resin and a charge-controlling agent. A volume average particle diameter X of the toner after a stress treatment satisfies Formula (1) below, and an amount Y of fine toner particles having particle diameters of 3 micrometers or smaller and circularity of 0.70 or less satisfies Formula (2) below.

$$6.0 \leq X(\text{micrometers}) \leq 8.5 \quad \text{Formula (1)}$$

$$Y(\% \text{ by mass}) \leq 4.3X(\text{micrometers}) - 14.6 \quad \text{Formula (2)}$$

The present inventors have found that fixing ability of a toner improved and background smear can be prevented even after the toner receives stress when a volume average particle diameter X of the toner after a stress treatment and an amount of the toner belongs to an ultra-fine powder region and irregularly shaped, i.e., an amount Y of fine toner particles having particle diameters of 3 micrometers or smaller and circularity of 0.70 or less, are specified.

When the volume average particle diameter X of the toner after a stress treatment is smaller than 6.0 micrometers, an amount of exposed surface of toner base particles increases, the toner particles tend to aggregate, and therefore white-missing spots in a solid image are formed in terms of image quality. When the volume average particle diameter X is greater than 8.5 micrometers, on the other hand, image quality in terms of dot reproducibility or fine line reproducibility is deteriorated.

The volume average particle diameter X of the toner after a stress treatment is more preferably 6.5 micrometers or greater but 8.0 micrometers or smaller.

When the amount of the toner belongs to an ultrafine powder region and irregularly shaped, i.e., an amount Y of

fine toner particles having particle diameters of 3 micrometers or smaller and circularity of 0.70 or less, is greater than the value of Formula (2), moreover, background smear occurs. The reason for occurrence of background smear is assumed as follows. Compared to spherical toner particles, irregular-shape toner particles have a large contact area with an electrostatic latent image bearer, such as a photoconductor and an amount of raw materials exposed to surfaces of toner base particles increases. Therefore, non-electrostatic adhesion of the toner to the photoconductor increases. Moreover, charge tends to be held in cavities of irregular-shape toner particles. Therefore, it is also considered that the photoconductor and projected portions of the irregular-shape toner particles are strongly adhered with electrostatic Coulomb force.

In the present disclosure, moreover, as well as the volume average particles X after the stress treatment satisfies Formula (1), the fine toner particle amount Y preferably satisfies Formula (3) below and more preferably satisfies Formula (4) below in view of an improvement of an effect obtainable by the present disclosure.

$$Y(\% \text{ by mass}) \leq 3.8X(\text{micrometers}) - 14.6 \quad \text{Formula (3)}$$

$$Y(\% \text{ by mass}) \leq 3.2X(\text{micrometers}) - 14.6 \quad \text{Formula (4)}$$

As the stress test for use in the present disclosure, the following treatment method is used in order to give a similar level of stress to stress applied in an actual device for evaluation.

Stress treatment: a container formed of polypropylene having a volume of 100 mL is charged with 5 g of the toner and 10 g of alumina beads having particle diameters of 0.5 mm and the toner is shaken by shaking the container using a shaker (YS-8D, available from YAYOI Co., Ltd.) with a stroke width of 80 mm, a stroke number of 250 times/min, and a shaking duration of 1 hour.

Under the treatment conditions having weaker stress than the above-described stress conditions, chipping or cracking of a toner is less likely to occur and stress applied is not similar to stress applied in an actual device. Therefore, an influence by the presence of an ultra-fine powder region cannot be confirmed.

Under the treatment conditions having stronger stress than the above-described stress conditions, stress stronger than stress applied in an actual device is applied to the toner. Therefore, an influence by the presence of an ultra-fine powder region cannot be confirmed.

Moreover, the toner of the present disclosure preferably includes a tetrahydrofuran (THF)-insoluble component in an amount of 10% by mass through 40% by mass. In a molecular-weight distribution of a THF-soluble component of the toner obtained by gel permeation chromatography (GPC), the toner preferably has a main peak between 10,000 and 16,000, and a molecular weight of a half-value width of the main peak is preferably 60,000 through 90,000. Within the THF-soluble component of the toner, a component having a molecular weight of 2,000 or less as determined by GPC is preferably from 15.0% by mass through 25.0% by mass and a component having a molecular weight of 100,000 or greater as determined by GPC is preferably 10.0% by mass or less.

Hot offset resistance can be improved by adjusting the THF-insoluble component to the range of 10% by mass through 40% by mass, namely making an absolute value of the THF-insoluble component of the toner smaller than an absolute value of the THF-soluble component.

Since the toner preferably has a main peak between 10,000 and 16,000 in the molecular-weight distribution of a THF-soluble component of the toner obtained by GPC, chipping or cracking of the toner can be prevented and moreover low-temperature fixing ability is improved.

When a half-value width of the main peak is molecular weight of less than 60,000, moreover, cracking or chipping of the toner may occur. When the half-value width of the main peak is molecular weight of greater than 90,000, low-temperature fixing ability may be deteriorated. Since a component having a molecular weight of 2,000 or less as determined by GPC is from 15.0% by mass through 25.0% by mass and a component having a molecular weight of 100,000 or greater as determined by GPC is 10.0% by mass or less within the THF-soluble component of the toner, low-temperature fixing ability is improved.

Next, materials used for the toner of the present disclosure will be described.

A binder resin for use in the present disclosure is not particularly limited, but the binder resin is preferably a polyester resin. The polyester resin is typically obtained through condensation polymerization between alcohol and carboxylic acid.

Examples of the alcohol include: glycols, such as ethylene glycol, diethylene glycol, triethylene glycol, and propylene glycol; etherified bisphenols, such as 1,4-bis(hydroxymethyl)cyclohexane and bisphenol A; other divalent alcohol monomers; and trivalent or higher polyvalent alcohol monomers.

Moreover, examples of the carboxylic acid include: divalent organic acid monomers, such as maleic acid, fumaric acid, phthalic acid, isophthalic acid, terephthalic acid, succinic acid, and malonic acid; and trivalent or higher polyvalent carboxylic acid monomers, such as 1,2,4-benzenetricarboxylic acid, 1,2,5-benzenetricarboxylic acid, 1,2,4-cyclohexanetricarboxylic acid, 1,2,4-naphthalenetricarboxylic acid, 1,2,5-hexanetricarboxylic acid, 1,3-dicarboxyl-2-methylenecarboxypropane, and 1,2,7,8-octanetetracarboxylic acid.

In view of thermal storage stability, the polyester resin is preferably a polyester resin having glass transition temperature Tg of 55 degrees Celsius or higher, more preferably a polyester resin having glass transition temperature Tg of 60 degrees Celsius or higher.

As described above, the polyester resin is preferably used as a resin component in the toner. Other resins may be used in combination as long as such resins do not adversely affect performance of the toner.

Examples of usable resins other than the polyester resin include the following resins.

Namely, examples of the usable resins include: styrene-based resins (homopolymers or copolymers including styrene or substituted styrene) such as polystyrene, chloropolystyrene, poly-alpha-methylstyrene, styrene/chlorostyrene copolymers, styrene/propylene copolymers, styrene/butadiene copolymers, styrene/vinyl chloride copolymers, styrene/vinyl acetate copolymers, styrene/maleic acid copolymers, styrene/acrylic acid ester copolymers (e.g., styrene/methyl acrylate copolymers, styrene/ethyl acrylate copolymers, styrene/butyl acrylate copolymers, styrene/octyl acrylate copolymers, and styrene/phenyl acrylate copolymers), styrene/methacrylic acid ester copolymers (e.g., styrene/methyl methacrylate copolymers, styrene/ethyl methacrylate copolymers, styrene/butyl methacrylate copolymers, and styrene/phenyl methacrylate copolymers), styrene/methyl alpha-chloroacrylate copolymers, and styrene/acrylonitrile/acrylic acid ester copolymers; vinyl chloride resins; styrene/vinyl

acetate copolymers; rosin-modified maleic acid resins; phenol resins; epoxy resins; polyethylene resins; polypropylene resins; ionomer resins; polyurethane resins; silicone resins; ketone resins; ethylene/ethyl acrylate copolymers; xylene resins; polyvinyl butyral resins; petroleum-based resins; and hydrogenated petroleum-based resins.

Production methods of the above-listed resins are not particularly limited, any of bulk polymerization, solution polymerization, emulsion polymerization, or suspension polymerization can be used.

Similarly to the polyester resin, moreover, glass transition temperature Tg of any of the resins above is preferably 55 degrees Celsius or higher and more preferably 60 degrees Celsius or higher, in view of thermal storage stability.

As a charge-controlling agent for use in the present disclosure, any charge-controlling agents known in the art, such as nigrosine dyes, metal complex salt dyes, and salicylic acid metal complexes, can be used alone or in combination. The charge-controlling agent is preferably a metal complex having trivalent or higher metal that may have a 6-coordination structure. Examples of the metal include Al, Fe, Cr, and Zr. Among the metal complex having trivalent or higher metal that may have a 6-coordination structure, a metal complex having Fe having no toxicity as a central metal is preferable. In the present disclosure, an amount of the charge-controlling agent is preferably 0.5 parts by mass or greater but 3.0 parts by mass or less relative to 100 parts by mass of the binder resin. When the amount of the charge-controlling agent is less than 0.5 parts by mass, a function of the charge-controlling agent is not sufficiently exhibited. When the amount of the charge-controlling agent is greater than 3.0 parts by mass, grindability of the toner is affected, hence blade adherence or filming on a photoconductor may be caused. Moreover, charging failures may be caused, and such a charging failure may be a cause for low image quality, such as toner supply failures and background smear. A more preferable amount of the charge-controlling agent is 1 part by mass or greater but 2.5 parts by mass or less relative to 100 parts by mass of the binder resin.

The charge-controlling agent for use in the present disclosure is preferably azo iron dyes represented by Structural Formula (1) below and/or Structural Formula (2) below because of excellent stress resistance.

[Chem. 1]



In Structural Formula (1), A<sup>+</sup> is an ammonium ion.

[Chem. 2]

Structural Formula (2)



In Structural Formula (2),  $J^+$  is H, an alkali metal, ammonium, alkyl ammonium ion, or a mixture of two or more of the above-listed substances.

Among the above-listed examples, the azo iron dye represented by Structural Formula (1) having appropriate charging ability and a high effect of improving background smear is preferably used.

The azo iron dye represented by Structural Formula (1) is available as T-77 and the azo iron dye represented by Structural Formula (2) is available as T-159 from Hodogaya Chemical Co., Ltd.

Examples of other preferable charge-controlling agents include zirconium salicylates. Zirconium salicylates are available from Hodogaya Chemical Co., Ltd.

As a colorant for use in the toner of the present disclosure, any dyes and pigments known in the art can be used alone or in combination. Examples of the dyes and pigments include carbon black, lamp black, iron black, aniline blue, phthalocyanine blue, phthalocyanine green, Hanza Yellow G, Rhodamine 6C lake, Calco Oil Blue, chrome yellow, quinacridone, benzidine yellow, rose bengal, and triallyl methane-based dyes. The toner can be used as a black color or full-color toners.

An amount of the colorant added is, for example, 1% by mass through 30% by mass and preferably 3% by mass through 20% by mass relative to the binder resin.

As a release agent for use in the toner of the present disclosure, any release agents known in the art can be used. Particularly, free fatty-acid carnauba wax, montan wax, and oxidized rice wax can be used alone or in combination.

The carnauba wax is suitably microcrystalline carnauba wax. The carnauba was is preferably carnauba wax having an acid value of 5 or less and gives particle diameters of 1 micrometer or smaller when the carnauba wax is dispersed in a toner binder.

The montan wax means montan-based wax typically refined from minerals. Similarly to the carnauba wax, the montan wax is preferably microcrystalline and preferably has an acid value of 5 through 14.

The oxidized rice wax is wax obtained by oxidizing rice bran wax in the air and preferably has an acid value of 10 through 30.

As other release agents, any of release agents known in the art, such as solid silicone varnish, higher fatty acid higher alcohol, montan-based ester wax, and low-molecular-weight polypropylene wax, can be used in combination.

An amount of the release agent(s) is, for example, 1 part by mass through 20 parts by mass and more preferably 2 parts by mass through 10 parts by mass relative to 100 parts by mass of the binder resin.

5 <Physical Properties Measuring Methods>

The above-mentioned various physical properties are measured in the following manner.

Volume Average Particle Diameter

A volume average particle diameter is determined by 10 performing a measurement by means of a particle-size analyzer ("Multisizer III," available from Beckman Coulter, Inc.) with an aperture diameter of 100 micrometers and analyzing using an analysis software (Beckman Coulter Multisizer 3, Version 3.51).

15 To 100 mL through 150 mL of an electrolyte aqueous solution, 0.1 mL through 5 mL of a 10% by mass surfactant (alkylbenzene sulfonate) is added. The electrolyte aqueous solution is an about 1% NaCl aqueous solution prepared by using first grade sodium chloride. For example, ISOTON-II 20 (available from Beckman Coulter, Inc.) can be used as the electrolyte aqueous solution. Subsequently, a measuring sample in an amount of 2 mg through 20 mg based on a solid content is added to the electrolyte aqueous solution, the resultant is dispersed for about 1 minute to about 3 minutes 25 by means of an ultrasonic disperser, and then a volume average particle diameter is measured by means of the analysis device with an aperture of 100 micrometers.

Circularity and Fine Toner Particle Amount

A measurement is performed using a flow particle image 30 analyzer (FPIA-3000, available from SYSMEX CORPORATION) and an analysis is performed using an analysis software. A sample is prepared for a measurement by adding 0.1 mL through 5 mL of a 10% by mass surfactant (alkylbenzene sulfonate) to about 50 mg of the toner and diluting 35 the resultant with 50 cc of ion-exchanged water to adjust a measurement concentration (count number) to 8,000 through 12,000. The circularity used in the present disclosure is an average circularity. As the fine toner particle amount, an amount (% by number) of particles having 40 particle diameters of 3.00 micrometers or smaller is calculated.

Molecular Weight Measurement (GPC)

A molecular weight is measured by gel permeation chromatography (GPC) under the following conditions.

Device: GPC-150C (available from WATERS)

Column: KF801 to 807 (available from SHODEX)

Temperature: 40 degrees Celsius

Solvent: tetrahydrofuran (THF)

Flow rate: 1.0 mL/min

50 Sample: A sample having a concentration of 0.05% through 0.6% in an amount of 0.1 mL is injected.

A number average molecular weight and a weight average molecular weight of the resin are calculated from a molecular weight distribution of the resin measured under the 55 above-described conditions using a molecular-weight calibration curve prepared from monodisperse polystyrene standard samples.

As for the polystyrene standard samples for preparing the calibration curve, Showdex STANDARD Std. Nos. S-7300, 60 S-210, S-390, S-875, S-1980, S-10.9, S-629, S-3.0, and S-0.580 available from SHOWA DENKO K.K. and toluene are used. As the detector, a refractive index (RI) detector is used.

THF-Soluble Component and THF-Insoluble Component

A toner is weighed by about 50 mg. To the toner, 10 g of THF is added to prepare a sufficiently dissolved toner solution. After separating through centrifugation, a super-

natant liquid is dried and a solid content of the supernatant liquid is calculated. The result is determined as a THF-soluble component. The value obtained by subtracting the THF-soluble component from a solid content of the entire toner is determined as a THF-insoluble component.

A production method of the toner of the present disclosure includes a melt-kneading step, a pulverizing step, and a classifying step. The melt-kneading step includes kneading toner materials with melting the toner materials to obtain a melt-kneaded product. The pulverizing step includes pulverizing the obtained melt-kneaded product to obtain a pulverized product. The classifying step includes classifying the pulverized product obtained by the pulverizing. A volume average particle diameter  $X$  of the toner after a stress treatment below satisfies Formula (1), and an amount  $Y$  of fine toner particles having particle diameters of 3 micrometers or smaller and circularity of 0.70 or less satisfies Formula (2).

In the melt-kneading, the toner materials are mixed, a melt-kneader is charged with the mixture to perform melt kneading. As the melt-kneader, for example, a single-screw or twin-screw continuous kneader, or a batch-type kneader using a roll mill can be used. For example, KTK twin-screw extruder available from Kobe Steel, Ltd., TEM twin-screw kneader available from TOSHIBA MACHINE CO., LTD., a mortar extruder available from KCK, PCM twin-screw extruder available from IKEGAI, and a co-kneader available from BUSS are suitably used. The melt kneading is preferably performed under appropriate conditions not to cut molecular chains of the binder resin. Specifically, the melt-kneading temperature is determined with reference to a softening point of the binder resin. When the melt-kneading temperature is excessively lower than the softening point, chain scission occurs significantly. When the melt-kneading temperature is too high, chain scission does not occur and therefore dispersion may not be progressed.

In the pulverizing step, the kneaded product obtained by the kneading is pulverized. In the pulverization, it is preferable that the kneaded product be roughly pulverized first, and then finely pulverized. At the time of the pulverization, a system where pulverization is performed by making the kneaded product crush into an impact board in a jet flow, particles are made crushed with each other in a jet flow to pulverize, or the kneaded product is pulverized with a narrow gap between a mechanically-rotating rotor and a stator.

The classifying step is to classify the pulverized product obtained by the pulverization to adjust to particles having the predetermined particle diameters. The classification can be performed by removing fine particle component by a cyclone, a decanter, or a centrifuge separator.

After completing the pulverizing step and the classifying step, the pulverized product is classified in an air flow by a centrifugal force etc., to thereby produce toner base particles having the predetermined particle diameters. Subsequently, external additives are optionally added to the toner base particles. The toner base particles and the external additives are mixed and stirred by a mixer to cover surfaces of the toner base particles with the external additive while crushing the external additives.

In order to achieve the characteristics of the present disclosure, "a volume average particle diameter  $X$  of the toner after a stress treatment satisfies Formula (1), and an amount  $Y$  of fine toner particles having particle diameters of 3 micrometers or smaller and circularity of 0.70 or less satisfies Formula (2)," an amount of fine particles of 3 micrometers or smaller itself may be reduced or circularity

of the fine particles can be adjusted to be outside the range of 0.70 or less. As a method for reducing the amount of fine particles, there is a method where two-stage classification or TTSP separator (available from HOSOKAWA MICRON 5 CORPORATION) where rotors are arranged in series are used. In order to increase circularity of fine particles, moreover, the adjustment can be achieved by circulating the toner in the pulverizing step through an increase in blower pressure or an increase in rotational speed using a rotor pulverizer.

Moreover, circularity can be also increased by performing pulverization several time at low rotational speed with a closed channel by means of a mechanical pulverizer.

Typically, one-component development tends to easily 15 apply stress to a toner and therefore the above-described problem of deterioration of image quality due to background smear is caused. The toner of the present disclosure can prevent deterioration of image quality even after the toner receives stress, and therefore the toner is particularly useful 20 as a toner for one-component development.

(Image Forming Method and Image Forming Apparatus)

An image forming method of the present disclosure includes forming an image by one-component development. The image forming method includes at least an electrostatic 25 latent image-forming step and a developing step, and may further include other steps, such as a charge-eliminating step, a cleaning step, a recycling step, and a controlling step, according to the necessity.

An image forming apparatus of the present disclosure 30 includes at least an electrostatic-latent-image bearer (may be referred to as a "photoconductor" hereinafter), an electrostatic latent image-forming unit configured to form an electrostatic latent image on the photoconductor, and a developing unit configured to develop the electrostatic latent image with a developer including a toner to form a visible image. The image forming apparatus may further include other units, such as a charge-eliminating unit, a cleaning unit, a recycling unit, and a controlling unit, according to the necessity.

40 The image forming method is preferably performed by the image forming apparatus. The electrostatic latent image-forming step can be preferably performed by the electrostatic latent image-forming unit, the developing step is preferably performed by the developing unit, and the above-mentioned other steps are preferably performed by the above-mentioned other units.

Electrostatic Latent Image-Forming Step and Electrostatic Latent Image-Forming Unit

The electrostatic latent image-forming step is a step 50 including forming an electrostatic latent image on an electrostatic-latent-image bearer.

A material, shape, structure, size, etc. of the electrostatic-latent-image bearer (may be also referred to as "electrophotographic photoconductor" or "photoconductor") are not 55 particularly limited and may be appropriately selected from materials, shapes, structures, sizes, etc., known in the art. A preferable example of the shape of the photoconductor is a drum shape. Examples of the material of the photoconductor include: inorganic photoconductors, such as amorphous silicon and selenium, and organic photoconductors (OPC), such as polysilane, and phthalopolymethine. Among the above-listed examples, an organic photoconductor (OPC) is preferable because an image of higher resolution can be obtained.

60 For example, formation of the electrostatic latent image can be performed by uniformly charging a surface of the electrostatic-latent-image bearer, followed by exposing the

## 11

surface of the electrostatic-latent-image bearer with light imagewise. The formation of the electrostatic latent image can be performed by an electrostatic latent image-forming unit.

For example, the electrostatic latent image-forming unit includes at least a charging unit (charger) configured to uniformly charge a surface of the electrostatic-latent-image bearer, and an exposing unit (exposure device) configured to expose the surface of the electrostatic-latent-image bearer to light imagewise.

For example, the charging can be performed by applying voltage to a surface of the electrostatic-latent-image bearer using the charger.

The charger is not particularly limited and may be appropriately selected depending on the intended purpose. Examples of the charger include a contact charger, known in the art as itself, equipped with an electroconductive or semiconductive roller, brush, film, or rubber blade, and a non-contact charger utilizing corona discharge, such as corotron, and scorotron.

The charger is preferably a charger that is disposed in contact with or without contact with the electrostatic-latent-image bearer and is configured to superimpose DC voltage and AC voltage to charge a surface of the electrostatic-latent-image bearer.

Moreover, the charger is preferably a charging roller disposed adjacent to the electrostatic-latent-image bearer via a gap tape without being in contact with the electrostatic-latent-image bearer, where a surface of the electrostatic-latent-image bearer is charged by applying superimposed DC and AC voltage to the charging roller.

The exposure can be performed by exposing the surface of the electrostatic-latent-image bearer to light imagewise using the exposure device.

The exposure device is not particularly limited as long as the exposure device can expose a surface of the electrostatic-latent-image bearer charged by the charger to light that is in the shape of an image to be formed. The exposure device may be appropriately selected depending on the intended purpose. Examples of the exposure device includes various exposure devices, such as a reproduction optical exposure device, a rod-lens array exposure device, a laser optical exposure device, and a liquid crystal shutter optical device.

In the present disclosure, a back light system where exposure is performed imagewise from a back side of the electrostatic-latent-image bearer may be employed.

## Developing Step and Developing Unit

The developing step is a step including developing the electrostatic latent image with the toner to form a visible image.

For example, formation of the visible image can be performed by developing the electrostatic latent image with the toner and can be performed by the developing unit.

For example, the developing unit is preferably a developing unit that stores the toner and includes at least a developing device capable of applying the toner to the electrostatic latent image in contact with the electrostatic latent image or without being in contact with the electrostatic latent image. The developing unit is more preferably a developing device equipped with a toner stored container.

The developing device may be a developing device for a single color or a developing device for multiple colors. Preferable examples of the developing device include a developing device including a stirrer configured to stir the toner to cause frictions to charge the toner, and a rotatable magnetic roller.

## 12

Inside the developing device, for example, the toner and the carrier are mixed and stirred to cause frictions, the toner is charged by the frictions, and the charged toner is held on a surface of the rotating magnetic roller in the form of a brush to thereby form a magnetic brush. Since the magnet roller is disposed adjacent to the electrostatic-latent-image bearer (photoconductor), part of the toner constituting the magnetic brush formed on the surface of the magnetic roller is transferred onto a surface of the electrostatic-latent-image bearer (photoconductor) by electric suction force. As a result, the electrostatic latent image is developed with the toner to form a visible image formed of the toner on the surface of the electrostatic-latent-image bearer (photoconductor).

## 15 Transferring Step and Transferring Unit

The transferring step is a step including transferring the visible image to a recording medium. A preferable embodiment of the transferring step is a step using an intermediate transfer member and including primary transferring a visible image onto the intermediate transfer member, followed by secondary transferring the visible image onto the recording medium. A more preferable embodiment of the transferring step is a step using, as the toner, toners of two or more colors, preferably full-color toners, and including a primary transferring step including transferring visible images onto an intermediate transfer member to form a composite transfer image, and a secondary transferring step including transferring the composite transfer image onto a recording medium.

20 The transfer can be performed by charging the visible image on the electrostatic-latent-image bearer (photoconductor) using a transfer charger. The transfer can be performed by the transfer unit. A preferable embodiment of the transferring unit is a transferring unit including a primary transferring unit configured to transfer visible images onto an intermediate transfer member to form a composite transfer image and a secondary transferring unit configured to transfer the composite transfer image onto a recording medium.

25 Note that, the intermediate transfer member is not particularly limited and may be appropriately selected from transfer members known in the art depending on the intended purpose. Preferable examples of the intermediate transfer member include a transfer belt.

30 The transferring unit (the primary transferring unit or the secondary transferring unit) preferably includes at least a transferring device configured to charge the visible image formed on the electrostatic-latent-image bearer (photoconductor) to release the visible image to the side of the recording medium. The number of the transferring device disposed may be one, or 2 or more.

35 Examples of the transferring device include a corona transfer device using corona discharge, a transfer belt, a transfer roller, a pressure-transfer roller, and an adhesion-transfer device.

40 Note that, the recording medium is not particularly limited and may be appropriately selected from recording media (recording paper) known in the art.

## Fixing Step and Fixing Unit

45 The fixing step is a step including fixing the transferred visible image onto the recording medium using a fixing device. The fixing step may be performed every time when the developer of each color is transferred onto the recording medium, or may be performed once when the developers of all colors are laminated.

50 The fixing device is not particularly limited and may be appropriately selected depending on the intended purpose.

## 13

The fixing device is preferably a heat-press unit. Examples of the heat-press unit include a combination of a heating roller and a press roller, and a combination of a heat roller, a press roller, and an endless belt.

The fixing device is preferably a unit that includes a heating body equipped with a heat generator, a film in contact with the heating body, and a press member pressed against the heating body via the film, and is configured to pass a recording medium on which an unfixed image is formed through between the film and the press member to heat-fixing the image onto the recording medium. Heating performed by the heat-press unit is generally preferably performed at 80 degrees Celsius through 200 degrees Celsius.

In the present disclosure, in combination with or instead of the fixing step and the fixing unit, for example, a photofixing device known in the art may be used depending on the intended purpose.

## Other Steps and Other Units

The charge-eliminating step is a step including applying charge-elimination bias to the electrostatic-latent-image bearer to eliminate the charge of the electrostatic-latent-image bearer. The charge-eliminating step is preferably performed by a charge-eliminating unit.

The charge-eliminating unit is not particularly limited as long as the charge-eliminating unit is capable of applying charge-elimination bias to the electrostatic-latent-image bearer. The charge-eliminating unit may be appropriately selected from charge eliminators known in the art. Examples of the charge-eliminating unit include charge-eliminating lamps.

The cleaning step is a step including removing the toner remained on the electrostatic-latent-image bearer. The cleaning step is preferably performed by a cleaning unit.

The cleaning unit is not particularly limited as long as the cleaning unit is capable of removing the toner remained on the electrostatic-latent-image bearer. The cleaning unit is appropriately selected from cleaners known in the art. Preferable examples of the cleaner include magnetic-brush cleaners, electrostatic-brush cleaners, magnetic-roller cleaners, blade cleaners, brush cleaners, and web cleaners.

The recycling step is a step including recycling the toner removed by the cleaning step to the developing unit. The recycling unit is preferably performed by a recycling unit. The recycling unit is not particularly limited. Examples of the recycling unit include conveying units known in the art.

The controlling step is a step including controlling each of the above-described steps. The controlling step is preferably performed by the controlling unit.

The controlling unit is not particularly limited as long as the controlling unit is capable of controlling operations of each of the above-mentioned units. The controlling unit may be appropriately selected depending on the intended purpose. Examples of the controlling unit include devices, such as sequencers and computers.

A first example of the image forming apparatus of the present disclosure is illustrated in FIG. 3. An image forming apparatus 100A includes a photoconductor drum 10, a charging roller 20, an exposing device, a developing device 40, an intermediate transfer belt 50, a cleaning device 60 including a cleaning blade, and a charge-eliminating lamp 70.

The intermediate transfer belt 50 is an endless belt that is supported with three rollers 51 disposed at the inner side of the intermediate transfer belt 50. The intermediate transfer belt 50 can be moved in the direction indicated with an arrow in FIG. 3. Part of the three rollers 51 also functions as

## 14

a transfer bias roller capable of applying transfer bias (primary transfer bias) to an intermediate transfer belt 50. Moreover, a cleaning device 90 having a cleaning blade is disposed adjacent to the intermediate transfer belt 50. Furthermore, a transfer roller 80 is disposed to face the intermediate transfer belt 50. The transfer roller is capable of applying transfer bias (secondary transfer bias) for transferring a toner image to transfer paper 95.

In the surrounding area of the intermediate transfer belt 50, a corona-charging device 58 configured to apply charge to the toner image transferred to the intermediate transfer belt 50 is disposed between a contact area of the photoconductor drum 10 and the intermediate transfer belt 50 and a contact area of the intermediate transfer belt 50 and the transfer paper 95 relative to a rotational direction of the intermediate transfer belt 50.

The developing device 40 includes a developing belt 41, and a black-developing unit 45K, a yellow-developing unit 45Y, a magenta-developing unit 45M, and a cyan-developing unit 45C disposed in the surrounding area of the developing belt 41. Note that, the developing unit of each color includes a developer-stored unit 42, a developer-supply roller 43, and a developing roller (developer bearer) 44. Moreover, the developing belt 41 is an endless belt supported by a plurality of belt rollers and is rotatable in the direction indicated with the arrow in FIG. 3. Moreover, part of the developing belt 41 is in contact with the photoconductor drum 10.

Next, a method for forming an image using the image forming apparatus 100A will be explained. First, a surface of the photoconductor drum 10 is uniformly charged using the charging roller 20, followed by applying exposure light L to the photoconductor drum 10 using an exposing device (not illustrated) to form an electrostatic latent image. Next, the electrostatic latent image forming on the photoconductor drum 10 is developed with a toner supplied from the developing device 40 to form a toner image. Moreover, the toner image formed on the photoconductor drum 10 is transferred (primary transfer) onto the intermediate transfer belt 50 by transfer bias applied from the roller 51, transferring the toner image (secondary transfer) onto transfer paper 95 by transfer bias applied from the transfer roller 80. Meanwhile, the toner remained on a surface of the photoconductor drum 10, from which the toner image has been transferred to the intermediate transfer belt 50, is removed by the cleaning device 60, followed by eliminating the charge from the surface using the charge-eliminating lamp 70.

A second example of the image forming apparatus for use in the present disclosure is illustrated in FIG. 4. The image forming apparatus 100B has the same structure to the structure of the image forming apparatus 100A, except that the developing belt 41 is not disposed, and the black-developing unit 45K, the yellow-developing unit 45Y, the magenta-developing unit 45M, and the cyan-developing unit 45C are disposed directly facing the perimeter of the photoconductor drum 10.

A third example of the image forming apparatus for use in the present disclosure is illustrated in FIG. 5. An image forming apparatus 100C is a tandem color-image forming apparatus and includes a photocopier main body 150, a paper-feeding table 200, a scanner 300, and an automatic document feeder (ADF) 400.

An intermediate transfer belt 50 disposed in a central area of the photocopier main body 150 is an endless belt supported by three rollers 14, 15, and 16. The intermediate transfer belt 50 can be rotated in the direction indicated with an arrow in FIG. 5.

the arrow in FIG. 5. A cleaning device 17 having a cleaning blade configured to remove a toner remained on the intermediate transfer belt 50, from which a toner image has been transferred to recording paper, is disposed adjacent to the roller 15. A yellow electrostatic-latent-image bearer 10Y, a cyan electrostatic-latent-image bearer 10C, a magenta electrostatic-latent-image bearer 10M, and a black electrostatic-latent-image bearer 10K are disposed parallel along the conveying direction, as well as facing the intermediate transfer belt 50 supported by the rollers 14 and 15.

Moreover, an exposing device 21 is disposed adjacent to the image forming unit 120. Furthermore, a secondary-transfer belt 24 is disposed at the side of the intermediate transfer belt 50 opposite to the side where the image forming unit 120 is disposed. Note that, the secondary-transfer belt 24 is an endless belt supported by a pair of rollers 23, and recording paper transported on the secondary-transfer belt 24 and the intermediate transfer belt 50 can be brought into contact with each other between the rollers 16 and 23.

Moreover, a fixing device 25 is disposed adjacent to the secondary-transfer belt 24. The fixing device 25 includes a fixing belt 26 that is an endless belt supported by a pair of rollers, and a press roller 27 disposed to be pressed against the fixing belt 26. Note that, a sheet reverser 28 configured to reverse recording paper when images are formed on both sides of the recording paper is disposed adjacent to the secondary-transfer belt 24 and the fixing device 25.

Next, a method for forming a full-color image using the image forming apparatus 100C will be explained. First, a color document is set on a document table 130 of the automatic document feeder (ADF) 400. Alternatively, the automatic document feeder 400 is opened, a color document is set on a contact glass 32 of a scanner 300 and then the automatic document feeder 400 is closed. In the case where the document is set on the automatic document feeder 400, once a start switch, which is not illustrated, is pressed, the document is transported onto the contact glass 32, and then the scanner 300 is driven to scan the document with a first carriage 33 equipped with a light source and a second carriage 34 equipped with a mirror. In the case where the document is set on the contact glass 32, the scanner 300 is immediately driven in the same manner as mentioned. Light is emitted from the first carriage 33 is reflected from a surface of the document and the reflected light is reflected by the second carriage 34, and then the reflected light is received by a reading sensor 36 via an image forming lens 35 to read the document to thereby obtain image information of black, yellow, magenta, and cyan.

Image information of each color is transmitted to a corresponding image-forming unit 18 of a corresponding image forming unit 120 to form a toner image of each color. As illustrated in FIG. 6, the image forming unit 120 of each color includes a photoconductor drum 10, a charging roller 160 configured to uniformly charge the photoconductor drum 10, an exposing device configured to apply exposure light L to the photoconductor drum 10 based on the image information of each color to form an electrostatic latent image of each color, a developing device 61 configured to develop the electrostatic latent image with a developer of each color to form a toner image of each color, a transfer roller 62 configured to transfer the toner image onto the intermediate transfer belt 50, a cleaning device 63 having a cleaning blade, and a charge-eliminating lamp 64.

The single-color toner images formed by the image forming units 120 of the above-mentioned colors are sequentially transferred (primary transfer) onto the intermediate transfer belt 50 moving with being supported by the rollers 14, 15,

and 16 to superimpose the single-color toner images to thereby form a composite toner image.

Meanwhile, one of paper feeding rollers 142 of the paper feeding table 200 is selectively rotated to feed sheets from one of vertically stacked paper feeding cassette 144 housed in a paper bank 143. The sheets are separated one another by a separation roller 145. The separated sheet is fed through a paper feeding path 146, then fed through a paper feeding path 148 in the photocopier main body 150 by conveying with a conveyance roller 147, and is stopped at a registration roller 49. Alternatively, paper feeding rollers are rotated to feed sheets on a bypass feeder 54. The sheets are separated one another by a separation roller 52. The separated sheet is fed through a manual paper feeding path 53, and is stopped at the registration roller 49.

Note that, the registration roller 49 is generally earthed at the time of use, but the registration roller 49 may be used in a state where bias is applied in order to remove paper dusts of recording paper. Next, the registration roller 49 is rotated to synchronously with the movement of the composite toner image formed on the intermediate transfer belt 50, to thereby send the recording paper between the intermediate transfer belt 50 and the secondary-transfer belt 24. The composite toner image is transferred (secondary transfer) on the recording paper. Note that, the toner remained on the intermediate transfer belt 50, from which the composite toner image has been transferred, is removed by the cleaning device 17.

The recording paper, onto which the composite toner image has been transferred, is conveyed by the secondary-transfer belt 24 and then the composite toner image is fixed by the fixing device 25. Next, the traveling path of the recording paper is changed by a switch craw 55 and the recording paper is ejected onto a paper-ejection tray 57 by an ejecting roller 56. Alternatively, the traveling path of the recording paper is changed by the switch craw 55 and the recording paper is reversed by the sheet reverser 28. After forming an image on a back side of the recording paper in the same manner, the recording paper is ejected onto the paper-ejection tray 57 by the ejection roller 56.

In the present disclosure, a toner stored unit is a unit that has a function of storing a toner and stores the toner therein. Examples of an embodiment of the toner stored unit include a toner stored container, a developing device, and a process cartridge.

The toner stored container is a container storing a toner. The developing device is a developing device including a developing unit storing a toner.

The process cartridge includes at least an electrostatic-latent-image bearer and a developing unit configured to develop an electrostatic latent image formed on the electrostatic-latent-image bearer with a developer to form a visible image. The process cartridge is detachably mounted in a main body of an image forming apparatus. The above-mentioned developer is the toner of the present disclosure. The process cartridge may further includes at least one selected from the group consisting of a charging unit, an exposing unit, and a cleaning unit.

Next, one embodiment of the process cartridge is illustrated in FIG. 2. As illustrated in FIG. 2, the process cartridge of the present embodiment includes an electrostatic-latent-image bearer 101 inside the process cartridge, includes a charging device 102, a developing device 104, and a cleaning unit 107, and may further include other units according to the necessity. In FIG. 2, the reference numeral 103 represents exposure from the exposing device and the reference numeral 105 represents recording paper.

As the electrostatic-latent-image bearer **101**, a similar electrostatic-latent-image bearer to the one used in the above-described image forming apparatus can be used. Moreover, an arbitrary charging member is used for the charging device **102**.

An image forming process performed by the process cartridge illustrated in FIG. 2 is as follows. While the electrostatic-latent-image bearer **101** is rotated clockwise, an electrostatic latent image corresponding to an exposure image is formed on a surface of the electrostatic-latent-image bearer **101** by performing charging by the charging device **102** and exposure **103** by an exposing unit (not illustrated).

The electrostatic latent image is developed with a toner by the developing device **104**, and the toner-developed image is transferred onto recording paper **105** by the transfer roller **108**, followed by printing out the recording paper. Subsequently, a surface of the electrostatic-latent-image bearer after the image transfer is cleaned by the cleaning unit **107**. Moreover, the charge of the surface of the electrostatic-latent-image bearer is eliminated by a charge-eliminating unit (not illustrated), and then the above-described operation of the image forming process is again repeated.

Since image formation is performed using the toner of the present disclosure by mounting the toner stored unit storing the toner of the present disclosure in the image forming apparatus, adhesion of the toner to a regulating blade is

inner atmosphere of the flask an inert atmosphere. Subsequently, 0.05 parts by mass of dibutyl tin oxide was added and the mixture inside the flask was allowed to react with maintaining the temperature to 200 degrees Celsius to thereby obtain each polyester. Various physical properties of each polyester are also presented in Tables 1 and 2. Note that, in Tables 1 and 2, the numerical values for the acid component and the alcohol component are represented by "part(s) by mass," "Mw" denotes a weight average molecular weight, and the numerical values for the THF-insoluble component are presented by "%."

TABLE 1

|                           | Polyester resin A       | Resin A-1 | Resin A-2 | Resin A-3 |
|---------------------------|-------------------------|-----------|-----------|-----------|
| 15<br>Acid component      | terephthalic acid       | 25        | 40        | 35        |
|                           | fumaric acid            | 10        |           | 30        |
|                           | succinic acid           | 10        | 15        |           |
| 20<br>Alcohol component   | trimellitic anhydride   |           |           |           |
|                           | bisphenol A(2.2)        | 20        | 35        | 25        |
|                           | propylene oxide         |           |           |           |
| 25<br>Physical properties | bisphenol A (2.2)       | 40        | 10        | 20        |
|                           | ethylene oxide          |           |           |           |
|                           | Mw                      | 35,000    | 60,000    | 42,000    |
|                           | peak-top                | 12,000    | 11,000    | 10,800    |
|                           | molecular weight        |           |           |           |
|                           | THF-insoluble component | 0         | 0         | 0         |

TABLE 2

|                     | Polyester resin B       | Resin B-1 | Resin B-2 | Resin B-3 | Resin B-4 | Resin B-5 |
|---------------------|-------------------------|-----------|-----------|-----------|-----------|-----------|
| Acid component      | terephthalic acid       | 22.5      | 15        | 20        | 35        | 22.5      |
|                     | fumaric acid            | 20        | 30        |           | 10        | 15        |
|                     | succinic acid           |           |           | 18        |           |           |
| Alcohol component   | trimellitic anhydride   | 20        | 30        | 10        | 35        | 15        |
|                     | bisphenol A (2.2)       | 20        | 30        | 15        | 25        | 30        |
|                     | propylene oxide         |           |           |           |           |           |
| Physical properties | bisphenol A (2.2)       | 20        | 15        | 25        | 15        | 15        |
|                     | ethylene oxide          |           |           |           |           |           |
|                     | Mw                      | 40,000    | 45,000    | 34,000    | 63,200    | 36,000    |
|                     | peak-top                | 13,000    | 9,500     | 12,000    | 17,000    | 15,200    |
|                     | molecular weight        |           |           |           |           |           |
|                     | THF-insoluble component | 25        | 38        | 19        | 45        | 10        |

inhibited, cleaning properties are sufficiently secured, and excellent image quality without background smear can be obtained.

## EXAMPLES

The present disclosure will be described in more detail by way of the following Examples. However, the present disclosure should not be construed as being limited to these Examples. Note that, "part(s)" mentioned in each Examples or Comparative Example denotes "part(s) by mass" unless otherwise stated.

### <Production of Polyester>

A four-necked recovery flask that had a volume of 1 L and was equipped with a thermometer, a stirrer, a condenser, and a nitrogen gas-inlet tube was charged with an acid component and an alcohol component presented in Tables 1 and 2. The flask was set in a heating mantle and the flask was heated in a state where nitrogen gas was introduced into the flask through the nitrogen gas-inlet tube to maintain the

### Example 1

50 Polyester resin A-1: 55.6 parts  
Polyester resin B-1: 44.4 parts  
Ric wax (TOWAX-3F16, available from TOA KASEI CO., LTD.): 3 parts  
55 Carbon black (#44, available from Mitsubishi Chemical Corporation): 6 parts  
Azo iron dye CCA1 (T-77, available from Hodogaya Chemical Co., Ltd.): 1.0 part by mass

After sufficiently stirring and mixing a mixture having the 60 composition above in Henschel Mixer, the resultant mixture was melt-kneaded by means of a twin-screw extrusion kneader (TEM-18SS, available from TOSHIBA MACHINE CO., LTD.). After cooling the obtained kneaded product to room temperature, the kneaded product was pulverized and 65 classified by means of a jet mill (IDS-2, available from NIPPON PNEUMATIC MFG. CO., LTD.) and a rotor classifier (50ATP, available from HOSOKAWA MICRON

19

CORPORATION), to thereby obtain toner base particles having a volume average particle diameter of 7.5 micrometers.

To 100 parts by mass of the obtained toner base particles, 2 parts by mass of HMDS-treated hydrophobic silica (RX200, available from NIPPON AEROSIL CO., LTD.) having an average particle diameter of 12 nm to thereby obtain Toner 1. Then, the above-described stress treatment was performed on Toner 1.

The volume average particle diameter X of Toner 1 after the stress treatment was 7.4 micrometers and an amount Y of fine toner particles having particle diameters of 3 micrometers or smaller and circularity of 0.70 or less was 8.6% by mass. Physical properties of the toner are presented in Table 3.

#### Example 2

Toner 2 was obtained in the same manner as in Example 1, except that Polyester Resin A-1 was changed to Polyester resin A-2, and 1.0 part of CCA1 of the charge-controlling agent was changed to 1.2 parts of CCA1. The volume average particle diameter X of Toner 2 after the stress treatment was 6.1 micrometers and the amount Y of fine toner particles was 0.9% by mass. Physical properties of the toner are presented in Table 3.

#### Example 3

Toner 3 was obtained in the same manner as in Example 1, except that Polyester Resin A-1 was changed to Polyester Resin A-2, Polyester Resin B-1 was changed to Polyester Resin B-2, and 1.0 part of CCA1 of the charge-controlling agent was changed to 1.5 parts of CCA1. The volume average particle diameter X of Toner 3 after the stress treatment was 8.4 micrometers and the amount Y of fine toner particles was 0.9% by mass. Physical properties of the toner are presented in Table 3.

#### Example 4

Toner 4 was obtained in the same manner as in Example 1, except that 55.6 parts of Polyester Resin A-1 was changed to 56.3 parts of Polyester Resin A-3, 44.4 parts of Polyester Resin B-1 was changed to 43.7 parts of Polyester Resin B-3, and 1.0 part of CCA1 of the charge-controlling agent was changed to 2.0 parts of CCA1. The volume average particle diameter X of Toner 4 after the stress treatment was 6.1 micrometers and the amount Y of fine toner particles was 11.6% by mass. Physical properties of the toner are presented in Table 3.

#### Example 5

Toner 5 was obtained in the same manner as in Example 1, except that 55.6 parts of Polyester Resin A-1 was changed to 54.2 parts of Polyester Resin A-3, 44.4 parts of Polyester Resin B-1 was changed to 45.8 parts of Polyester Resin B-3, and 1.0 part of CCA1 of the charge-controlling agent was changed to 1.4 parts of CCA1. The volume average particle diameter X of Toner 5 after the stress treatment was 8.4 micrometers and the amount Y of fine toner particles was 21.5% by mass. Physical properties of the toner are presented in Table 3.

#### Example 6

Toner 6 was obtained in the same manner as in Example 1, except that 55.6 parts of Polyester Resin A-1 was changed

20

to 56.0 parts, 44.4 parts of Polyester Resin B-1 was changed to 44.0 parts, and 1.0 part of CCA1 of the charge-controlling agent was changed to 1.7 parts of CCA1. The volume average particle diameter X of Toner 6 after the stress treatment was 6.1 micrometers and the amount Y of fine toner particles was 11.6% by mass. Physical properties of the toner are presented in Table 3.

#### Example 7

Toner 7 was obtained in the same manner as in Example 1, except that 55.6 parts of Polyester Resin A-1 was changed to 54.5 parts and 44.4 parts of Polyester Resin B-1 was changed to 45.5 parts. The volume average particle diameter X of Toner 7 after the stress treatment was 8.4 micrometers and the amount Y of fine toner particles was 21.5% by mass. Physical properties of the toner are presented in Table 3.

#### Example 8

Toner 8 was obtained in the same manner as in Example 1, except that Polyester Resin B-1 was changed to Polyester Resin B-4 and 1.0 part of CCA1 of the charge-controlling agent was changed to 1.3 parts of CCA1. The volume average particle diameter X of Toner 8 after the stress treatment was 7.4 micrometers and the amount Y of fine toner particles was 16.8% by mass. A THF-insoluble component of Toner 8 was measured and the result was 8.0%. Physical properties of the toner are presented in Table 3.

#### Example 9

Toner 9 was obtained in the same manner as in Example 1, except that Polyester Resin B-1 was changed to Polyester Resin B-5 and 1.0 part of CCA1 of the charge-controlling agent was changed to 0.9 parts of CCA1. The volume average particle diameter X of Toner 9 after the stress treatment was 7.4 micrometers and the amount Y of fine toner particles was 16.8% by mass. A THF-insoluble component of Toner 9 was measured and the result was 42.0%. Physical properties of the toner are presented in Table 3.

#### Example 10

Toner 10 was obtained in the same manner as in Example 1, except that 1.0 part of CCA1 of the charge-controlling agent was changed to 0.4 parts of CCA2 (TN-105, available from Hodogaya Chemical Co., Ltd.). The volume average particle diameter X of Toner 10 after the stress treatment was 7.4 micrometers and the amount Y of fine toner particles was 16.8% by mass. Physical properties of the toner are presented in Table 3.

#### Example 11

Toner 11 was obtained in the same manner as in Example 1, except that 1.0 part of CCA1 of the charge-controlling agent was changed to 3.1 parts of CCA2 (zirconium salicylate, TN-105, available from Hodogaya Chemical Co., Ltd.). The volume average particle diameter X of Toner 11 after the stress treatment was 7.4 micrometers and the amount Y of fine toner particles was 16.8% by mass. Physical properties of the toner are presented in Table 3.

#### Comparative Example 1

Comparative Toner 1 was obtained in the same manner as in Example 1, except that 55.6 parts of Polyester Resin A-1

was changed to 54.0 parts and 44.4 parts of Polyester Resin B-1 was changed to 46.0 parts. The volume average particle diameter X of Comparative Toner 1 after the stress treatment was 5.9 micrometers and the amount Y of fine toner particles was 0.7% by mass. Physical properties of the toner are presented in Table 3.

## Comparative Example 2

In Comparative Example 1, the pulverization classification conditions were changed to give the volume average diameter X after the stress treatment of 8.6 micrometers and the fine toner particle amount Y of 1.2% by mass (Comparative Toner 2). Physical properties of the toner are presented in Table 3.

## Comparative Example 3

Comparative Toner 3 was obtained in the same manner as in Example 1, except that 55.6 parts of Polyester Resin A-1 was changed to 57.2 parts and 44.4 parts of Polyester Resin B-1 was changed to 42.8 parts. The volume average particle diameter X of Comparative Toner 3 after the stress treatment was 5.9 micrometers and the amount Y of fine toner particles was 10.6% by mass. Physical properties of the toner are presented in Table 3.

## Comparative Example 4

In Comparative Example 3, the pulverization classification conditions were changed to give the volume average diameter X after the stress treatment of 8.6 micrometers and the fine toner particle amount Y of 22.2% by mass (Comparative Toner 4). Physical properties of the toner are presented in Table 3.

## Comparative Example 5

Comparative Toner 5 was obtained in the same manner as in Example 1, except that 55.6 parts of Polyester Resin A-1 was changed to 56.5 parts and 44.4 parts of Polyester Resin B-1 was changed to 43.5 parts. The volume average particle diameter X of Comparative Toner 5 after the stress treatment was 6.1 micrometers and the amount Y of fine toner particles was 11.8% by mass. Physical properties of the toner are presented in Table 3.

## Comparative Example 6

In Comparative Example 5, the pulverization classification conditions were changed to give the volume average diameter X after the stress treatment of 8.4 micrometers and the fine toner particle amount Y of 22.3% by mass (Comparative Toner 6).

Physical properties of the toner are presented in Table 3.

TABLE 3

| Resin       |        |         |        | Physical properties of toner |                              |                  |                  |
|-------------|--------|---------|--------|------------------------------|------------------------------|------------------|------------------|
| Rosin A     |        | Resin B |        | Particle diameter            | Fine toner particle amount Y |                  |                  |
| Type        | Amount | Type    | Amount |                              | Formula 2                    | Formula 3        | Formula 4        |
| Ex. 1       | A-1    | 55.6    | B-1    | 44.4                         | 7.4                          | satisfied        | satisfied        |
| Ex. 2       | A-2    | 55.6    | B-1    | 44.4                         | 6.1                          | satisfied        | satisfied        |
| Ex. 3       | A-2    | 55.6    | B-2    | 44.4                         | 8.4                          | satisfied        | satisfied        |
| Ex. 4       | A-3    | 56.3    | B-3    | 43.7                         | 6.1                          | satisfied        | over upper limit |
| Ex. 5       | A-3    | 64.2    | B-3    | 46.8                         | 8.4                          | satisfied        | over upper limit |
| Ex. 6       | A-1    | 56.0    | B-1    | 44.0                         | 6.1                          | satisfied        | over upper limit |
| Ex. 7       | A-1    | 64.6    | B-1    | 48.6                         | 8.4                          | satisfied        | over upper limit |
| Ex. 8       | A-1    | 55.6    | B-4    | 44.4                         | 7.4                          | satisfied        | satisfied        |
| Ex. 9       | A-1    | 65.6    | B-5    | 44.4                         | 7.4                          | satisfied        | satisfied        |
| Ex. 10      | A-1    | 55.6    | B-1    | 44.4                         | 7.4                          | satisfied        | satisfied        |
| Ex. 11      | A-1    | 55.6    | B-1    | 44.4                         | 7.4                          | satisfied        | satisfied        |
| Comp. Ex. 1 | A-1    | 54.0    | B-1    | 46.0                         | 5.9                          | satisfied        | satisfied        |
| Comp. Ex. 2 | A-1    | 54.0    | B-1    | 46.0                         | 8.6                          | satisfied        | satisfied        |
| Comp. Ex. 3 | A-1    | 57.2    | B-1    | 42.8                         | 5.9                          | satisfied        | satisfied        |
| Comp. Ex. 4 | A-1    | 57.2    | B-1    | 42.8                         | 8.6                          | satisfied        | satisfied        |
| Comp. Ex. 5 | A-1    | 56.5    | B-1    | 43.6                         | 6.1                          | over upper limit | over upper limit |
| Comp. Ex. 6 | A-1    | 56.5    | B-1    | 43.6                         | 8.4                          | over upper limit | over upper limit |

## Physical properties of toner

| THF    | Main | THF soluble component (Mw)   |                       |                  | Charge-controlling agent                      |                                                 |                       |          |
|--------|------|------------------------------|-----------------------|------------------|-----------------------------------------------|-------------------------------------------------|-----------------------|----------|
|        |      | insoluble component (mass %) | peak molecular weight | Half-value width | Amount of component of 2,000 or less (mass %) | Amount of component of 100,000 or more (mass %) | Azo iron dye part (a) |          |
| Ex. 1  | 26   | 11,700                       | 72,600                | 22.3             | 6.1                                           | CCA1                                            | 1.0                   | Toner 1  |
| Ex. 2  | 26   | 11,700                       | 72,600                | 22.3             | 6.1                                           | CCA1                                            | 1.2                   | Toner 2  |
| Ex. 3  | 35   | 14,200                       | 77,400                | 24.0             | 8.6                                           | CCA1                                            | 1.5                   | Toner 3  |
| Ex. 4  | 18   | 11,050                       | 72,200                | 21.8             | 6.3                                           | CCA1                                            | 2.0                   | Toner 4  |
| Ex. 5  | 24   | 12,100                       | 71,800                | 22               | 6.4                                           | CCA1                                            | 1.4                   | Toner 5  |
| Ex. 6  | 24   | 12,100                       | 71,800                | 22               | 6.4                                           | CCA1                                            | 1.7                   | Toner 6  |
| Ex. 7  | 13   | 11,000                       | 69,800                | 18.9             | 6.1                                           | CCA1                                            | 1.0                   | Toner 7  |
| Ex. 8  | 8    | 9,000                        | 55,000                | 14               | 11                                            | CCA1                                            | 1.3                   | Toner 8  |
| Ex. 9  | 42   | 16,500                       | 90,500                | 26               | 11                                            | CCA1                                            | 0.9                   | Toner 9  |
| Ex. 10 | 26   | 11,700                       | 72,600                | 22.3             | 6.1                                           | CCA2                                            | 0.4                   | Toner 10 |
| Ex. 11 | 26   | 11,700                       | 72,600                | 22.3             | 6.1                                           | CCA2                                            | 3.1                   | Toner 11 |

TABLE 3-continued

|             |    |        |        |      |     |      |     |               |
|-------------|----|--------|--------|------|-----|------|-----|---------------|
| Comp. Ex. 1 | 26 | 11,700 | 72,000 | 22.3 | 6.1 | CCA1 | 1.0 | Comp. Toner 1 |
| Comp. Ex. 2 | 26 | 11,700 | 72,600 | 22.8 | 6.1 | CCA1 | 1.0 | Comp. Toner 2 |
| Comp. Ex. 3 | 35 | 14,200 | 77,400 | 24.0 | 8.6 | CCA1 | 1.0 | Comp. Toner 3 |
| Comp. Ex. 4 | 35 | 14,200 | 77,400 | 24.0 | 8.6 | CCA1 | 1.0 | Comp. Toner 4 |
| Comp. Ex. 5 | 24 | 11,500 | 71,800 | 22   | 6.4 | CCA1 | 1.0 | Comp. Toner 5 |
| Comp. Ex. 6 | 24 | 11,500 | 71,800 | 22   | 6.4 | CCA1 | 1.0 | Comp. Toner 6 |

The following evaluations were performed on the obtained toners after the stress treatment.

<Evaluation Methods>

1. Fixing Ability

(Low-Temperature Fixing Ability)

IPSiO SP C220 available from Ricoh Company Limited was modified and the modified device was charged with the toner. The device was set in a manner that an amount of the toner deposition on Type 6000T paper available from Ricoh Company Limited was to be 10 g/m<sup>2</sup>, and the paper on which an unfixed square solid image having a side of 40 mm was formed was prepared.

Next, the prepared unfixed solid image was passed through a modified fixing unit of IPSiO SP 4510SF available from Ricoh Company Limited with setting the system speed to 240 mm/sec, to thereby fix the image.

The test was performed by varying the fixing temperature from 120 degrees Celsius through 160 degrees Celsius by 5 degrees Celsius. The output images were visually observed and the temperature at which unintentional toner transfer did not occur on the white background region was determined as the minimum fixing temperature.

A: the minimum fixing temperature was lower than 140 degrees Celsius

B: the minimum fixing temperature was 140 degrees Celsius or higher but lower than 150 degrees Celsius

C: the minimum fixing temperature was 150 degrees Celsius or higher but lower than 160 degrees Celsius

D: the minimum fixing temperature was 160 degrees Celsius or higher

(High-Temperature Release Ability)

IPSiO SP C220 available from Ricoh Company Limited was modified. The modified device was charged with the toner. An unfixed square-solid image having a side of 40 mm was printed on Type 6000T available from Ricoh Company Limited by setting the device in a manner that a deposition amount was to be 10 g/m<sup>2</sup>.

Next, the prepared unfixed solid image was passed through the modified fixing unit of IPSiO SP 4510SF available from Ricoh Company Limited with setting the system speed to 240 mm/sec to thereby fix the image.

The test was performed by varying the fixing temperature from 160 degrees Celsius through 220 degrees Celsius by 5 degrees Celsius. The output images were visually observed and the temperature at which unintentional toner transfer did not occur on the white background region was determined as the maximum fixing temperature.

A: the maximum fixing temperature was 210 degrees Celsius or higher

B: the maximum fixing temperature was 190 degrees Celsius or higher but lower than 210 degrees Celsius

C: the maximum fixing temperature was 170 degrees Celsius or higher but lower than 190 degrees Celsius

D: the maximum fixing temperature was lower than 170 degrees Celsius

2. Evaluation of Background Smear

IPSiO SP C220 available from Ricoh Company Limited was modified. The modified device was charged with 13.5 g of the above-obtained toner, and SCOTCH TAPE was adhered to an entire surface of an exposed area of a photoconductor operation of which was suspended during printing of a blank sheet. The peeled SCOTCH TAPE was adhered to Type 6000T paper available from Ricoh Company Limited and was then stored.

A value of L\* on the tape was measured by X-rite.

A: L\* was 91 or greater

B: L\* was 89 or greater but less than 91

C: L\* was 85 or greater but less than 89

D: L\* was less than 85

3. Evaluation of Blade-Adherence Resistance

A developing unit of IPSiO SPC220 available from Ricoh Company Limited was charged with 20 g of the toner and a blade-adherence evaluation was performed by means of an external idle machine. The blade adherence was confirmed every 5 minutes by visually observing lines derived from the adherence in the areas of the developing roller at the image forming section where each area was from each edge of the developing roller to a position that was 5 cm from the edge. Evaluation criteria are as described below.

The following criteria judge the time when blade adherence occurred.

A: 120 minutes or later

B: 60 minutes or later but before 120 minutes

C: 30 minutes or later but before 60 minutes

D: before 30 minutes

4. Image Evaluation

IPSiO SP C220 available from Ricoh Company Limited was modified and the modified device was charged with 13.5 g of the toner. An evaluation image was output and a rank evaluation was performed on the evaluation image according to a criteria sample for white missing spots in a solid image and a criteria sample for dot reproducibility.

A: Rank 4 or higher

B: Rank 3 or higher but lower than Rank 4

C: Rank 2 or higher but lower than Rank 3

D: Lower than Rank 2

The evaluation results are presented in Table 4.

TABLE 4

| Fixing ability                 |        |            |                                  |            |                  |            |
|--------------------------------|--------|------------|----------------------------------|------------|------------------|------------|
| low temperature fixing ability |        |            | high-temperature release ability |            | Background smear |            |
|                                | (° C.) | evaluation | (° C.)                           | evaluation | L*               | evaluation |
| Toner 1                        | 138    | A          | 220                              | A          | 93.0             | A          |
| Toner 2                        | 141    | B          | 195                              | B          | 94.0             | A          |
| Toner 3                        | 143    | B          | 210                              | A          | 94.5             | A          |
| Toner 4                        | 148    | B          | 215                              | A          | 88.0             | C          |

TABLE 4-continued

| Blade adherence resistance |            |      |                     |      |                                 |      | Image evaluation |            |      |            |      |            |
|----------------------------|------------|------|---------------------|------|---------------------------------|------|------------------|------------|------|------------|------|------------|
| evaluation                 |            |      | white missing spots |      | dot reproducibility (fine line) |      | time [min]       | evaluation | rank | evaluation | rank | evaluation |
| time [min]                 | evaluation | rank | evaluation          | rank | evaluation                      | rank |                  |            |      |            |      |            |
| Toner 1                    | 120        | A    | 5                   | A    | 3.5                             | B    |                  |            |      |            |      |            |
| Toner 2                    | 75         | B    | 2.5                 | C    | 4                               | A    |                  |            |      |            |      |            |
| Toner 3                    | 110        | B    | 3                   | B    | 3                               | B    |                  |            |      |            |      |            |
| Toner 4                    | 70         | B    | 2                   | C    | 3                               | B    |                  |            |      |            |      |            |
| Toner 5                    | 115        | B    | 3.5                 | B    | 2                               | C    |                  |            |      |            |      |            |
| Toner 6                    | 115        | B    | 2.5                 | C    | 3.5                             | B    |                  |            |      |            |      |            |
| Toner 7                    | 80         | B    | 3.5                 | B    | 3.5                             | B    |                  |            |      |            |      |            |
| Toner 8                    | 45         | C    | 4                   | A    | 3                               | B    |                  |            |      |            |      |            |
| Tones 9                    | 120        | A    | 4.5                 | A    | 2.5                             | C    |                  |            |      |            |      |            |
| Toner 10                   | 50         | C    | 4                   | A    | 3                               | B    |                  |            |      |            |      |            |
| Toner 11                   | 120        | A    | 2                   | C    | 3                               | B    |                  |            |      |            |      |            |
| Comp. Toner 1              | 110        | B    | 1.5                 | D    | 3                               | B    |                  |            |      |            |      |            |
| Comp. Toner 2              | 50         | C    | 3                   | B    | 1.5                             | D    |                  |            |      |            |      |            |
| Comp. Toner 3              | 105        | B    | 1.5                 | D    | 2                               | C    |                  |            |      |            |      |            |
| Comp. Toner 4              | 70         | B    | 3.5                 | B    | 1                               | D    |                  |            |      |            |      |            |
| Comp. Toner 5              | 40         | C    | 3.5                 | B    | 3                               | B    |                  |            |      |            |      |            |
| Comp. Toner 6              | 55         | C    | 3                   | B    | 3.5                             | B    |                  |            |      |            |      |            |

It was found from the results of Table 4 that the toner of the present disclosure had excellent fixing ability and could prevent deterioration of image quality due to background smear even after the toner received stress, compared to the comparative toners. FIG. 1 is a graph depicting a relationship between the volume average particle diameter X of the toner after the stress treatment and the fine toner particle amount Y. The area surrounded by the solid line is a range specified by the present disclosure. Examples satisfied Formula 4 exhibited particularly excellent results.

## REFERENCE SIGNS LIST

|      |                                                         |    |      |                            |
|------|---------------------------------------------------------|----|------|----------------------------|
| 10:  | electrostatic-latent-image bearer (photoconductor drum) | 35 | 32:  | contact glass              |
| 10K: | electrostatic-latent-image bearer for black             | 50 | 33:  | first carriage             |
| 10Y: | electrostatic-latent-image bearer for yellow            |    | 34:  | second carriage            |
| 10M: | electrostatic-latent-image bearer for magenta           |    | 35:  | image forming lens         |
| 10C: | electrostatic-latent-image bearer for cyan              |    | 36:  | reading sensor             |
| 14:  | roller                                                  | 40 | 40:  | developing device          |
| 15:  | roller                                                  |    | 41:  | developing belt            |
| 16:  | roller                                                  |    | 42K: | developer-stored unit      |
| 17:  | cleaning device                                         |    | 42Y: | developer-stored unit      |
| 18:  | image-forming unit                                      |    | 42M: | developer-stored unit      |
| 20:  | charging roller                                         |    | 42C: | developer-stored unit      |
| 21:  | exposing device                                         | 45 | 43K: | developer-supply roller    |
| 22:  | secondary transferring device                           |    | 43Y: | developer-supply roller    |
| 23:  | roller                                                  |    | 43M: | developer-supply roller    |
| 24:  | secondary-transfer belt                                 |    | 43C: | developer-supply roller    |
| 25:  | fixing device                                           |    | 44K: | developing roller          |
| 26:  | fixing belt                                             |    | 44Y: | developing roller          |
| 27:  | press roller                                            |    | 44M: | developing roller          |
| 28:  | sheet reverser                                          |    | 44C: | developing roller          |
|      |                                                         |    | 45K: | black developing unit      |
|      |                                                         |    | 45Y: | yellow developing unit     |
|      |                                                         |    | 45M: | magenta developing unit    |
|      |                                                         |    | 45C: | cyan developing unit       |
|      |                                                         |    | 49:  | registration roller        |
|      |                                                         |    | 50:  | intermediate transfer belt |
|      |                                                         |    | 51:  | roller                     |
|      |                                                         |    | 52:  | separation roller          |
|      |                                                         |    | 53:  | manual paper feeding path  |
|      |                                                         |    | 54:  | bypass feeder              |
|      |                                                         |    | 55:  | switch crav                |
|      |                                                         |    | 56:  | ejection roller            |
|      |                                                         |    | 57:  | paper ejection tray        |
|      |                                                         |    | 58:  | corona-charging device     |

- 60: cleaning device  
 61: developing device  
 62: transfer roller  
 63: cleaning device  
 64: charge-eliminating lamp  
 70: charge-eliminating lamp  
 80: transfer roller  
 90: cleaning device  
 95: transfer paper  
 100A, 100B, 100C: image forming device  
 101: electrostatic-latent-image bearer  
 102: charging device  
 103: exposure from exposing device  
 104: developing device  
 105: recording paper  
 107: cleaning unit  
 108: transfer roller  
 120: image forming unit  
 130: document table  
 142: paper feeding roller  
 143: paper bank  
 144: paper feeding cassette  
 145: separation roller  
 146: paper feeding path  
 147: conveyance roller  
 148: paper feeding path  
 150: photocopier main body  
 160: charging roller  
 200: paper feeding table  
 300: scanner  
 400: automatic document feeder (ADF)

The invention claimed is:

1. A toner comprising:  
 a binder resin; and  
 a charge-controlling agent,  
 wherein a volume average particle diameter X of the toner  
 after a stress treatment below satisfies Formula (1)  
 below, and  
 an amount Y of fine toner particles having particle diameters of 3 micrometers or smaller and circularity of 0.70  
 or less satisfies Formula (2) below,

$$6.0 \leq X(\text{micrometers}) \leq 8.5$$

Formula (1)

$$Y(\%) \leq 4.3X(\text{micrometers}) - 14.6$$

Formula (2)

where the stress treatment includes charging a container formed of polypropylene having a volume of 100 mL with 5 g of the toner and 10 g of alumina beads having particle diameters of 0.5 mm, and shaking the toner by shaking the container using a shaker (YS-8D, available from YAYOI Co., Ltd.) with a stroke width of 80 mm, a stroke number of 250 times/min, and a shaking duration of 1 hour.

2. The toner according to claim 1,  
 wherein the amount Y of the fine toner particles satisfies  
 Formula (3) below,

$$Y(\%) \leq 3.8X(\text{micrometers}) - 14.6$$

Formula (3)

3. The toner according to claim 1,  
 wherein the amount Y of the fine toner particles satisfies  
 Formula (4) below,  

$$Y(\%) \leq 3.2X(\text{micrometers}) - 14.6$$
Formula (4)
- 5
4. The toner according to claim 1,  
 wherein the charge-controlling agent includes an azo iron  
 dye.
- 10
5. The toner according to claim 1,  
 wherein the toner includes a THF-insoluble component in  
 an amount of 10% by mass through 40% by mass,  
 a molecular-weight distribution of a THF-soluble com-  
 ponent of the toner obtained by gel permeation chro-  
 matography (GPC) has a main peak between 10,000  
 and 16,000, where a half-value width of the main peak  
 is a molecular weight of 60,000 through 90,000, and  
 within the THF-soluble component of the toner, a com-  
 ponent having a molecular weight of 2,000 or less as  
 determined by GPC is from 15.0% by mass through  
 25.0% by mass and a component having a molecular  
 weight of 100,000 or greater as determined by GPC is  
 10.0% by mass or less.
- 15
6. A toner production method comprising:  
 kneading toner materials with melting the toner materials  
 to obtain a melt-kneaded product;  
 pulverizing the melt-kneaded product to obtain a pulver-  
 20  
 25  
 30  
 35  
 40  
 45  
 50  
 55  
 60  
 65  
 70  
 75  
 80  
 85  
 90  
 95  
 100  
 105  
 110  
 115  
 120  
 125  
 130  
 135  
 140  
 145  
 150  
 155  
 160  
 165  
 170  
 175  
 180  
 185  
 190  
 195  
 200  
 205  
 210  
 215  
 220  
 225  
 230  
 235  
 240  
 245  
 250  
 255  
 260  
 265  
 270  
 275  
 280  
 285  
 290  
 295  
 300  
 305  
 310  
 315  
 320  
 325  
 330  
 335  
 340  
 345  
 350  
 355  
 360  
 365  
 370  
 375  
 380  
 385  
 390  
 395  
 400  
 405  
 410  
 415  
 420  
 425  
 430  
 435  
 440  
 445  
 450  
 455  
 460  
 465  
 470  
 475  
 480  
 485  
 490  
 495  
 500  
 505  
 510  
 515  
 520  
 525  
 530  
 535  
 540  
 545  
 550  
 555  
 560  
 565  
 570  
 575  
 580  
 585  
 590  
 595  
 600  
 605  
 610  
 615  
 620  
 625  
 630  
 635  
 640  
 645  
 650  
 655  
 660  
 665  
 670  
 675  
 680  
 685  
 690  
 695  
 700  
 705  
 710  
 715  
 720  
 725  
 730  
 735  
 740  
 745  
 750  
 755  
 760  
 765  
 770  
 775  
 780  
 785  
 790  
 795  
 800  
 805  
 810  
 815  
 820  
 825  
 830  
 835  
 840  
 845  
 850  
 855  
 860  
 865  
 870  
 875  
 880  
 885  
 890  
 895  
 900  
 905  
 910  
 915  
 920  
 925  
 930  
 935  
 940  
 945  
 950  
 955  
 960  
 965  
 970  
 975  
 980  
 985  
 990  
 995  
 1000  
 1005  
 1010  
 1015  
 1020  
 1025  
 1030  
 1035  
 1040  
 1045  
 1050  
 1055  
 1060  
 1065  
 1070  
 1075  
 1080  
 1085  
 1090  
 1095  
 1100  
 1105  
 1110  
 1115  
 1120  
 1125  
 1130  
 1135  
 1140  
 1145  
 1150  
 1155  
 1160  
 1165  
 1170  
 1175  
 1180  
 1185  
 1190  
 1195  
 1200  
 1205  
 1210  
 1215  
 1220  
 1225  
 1230  
 1235  
 1240  
 1245  
 1250  
 1255  
 1260  
 1265  
 1270  
 1275  
 1280  
 1285  
 1290  
 1295  
 1300  
 1305  
 1310  
 1315  
 1320  
 1325  
 1330  
 1335  
 1340  
 1345  
 1350  
 1355  
 1360  
 1365  
 1370  
 1375  
 1380  
 1385  
 1390  
 1395  
 1400  
 1405  
 1410  
 1415  
 1420  
 1425  
 1430  
 1435  
 1440  
 1445  
 1450  
 1455  
 1460  
 1465  
 1470  
 1475  
 1480  
 1485  
 1490  
 1495  
 1500  
 1505  
 1510  
 1515  
 1520  
 1525  
 1530  
 1535  
 1540  
 1545  
 1550  
 1555  
 1560  
 1565  
 1570  
 1575  
 1580  
 1585  
 1590  
 1595  
 1600  
 1605  
 1610  
 1615  
 1620  
 1625  
 1630  
 1635  
 1640  
 1645  
 1650  
 1655  
 1660  
 1665  
 1670  
 1675  
 1680  
 1685  
 1690  
 1695  
 1700  
 1705  
 1710  
 1715  
 1720  
 1725  
 1730  
 1735  
 1740  
 1745  
 1750  
 1755  
 1760  
 1765  
 1770  
 1775  
 1780  
 1785  
 1790  
 1795  
 1800  
 1805  
 1810  
 1815  
 1820  
 1825  
 1830  
 1835  
 1840  
 1845  
 1850  
 1855  
 1860  
 1865  
 1870  
 1875  
 1880  
 1885  
 1890  
 1895  
 1900  
 1905  
 1910  
 1915  
 1920  
 1925  
 1930  
 1935  
 1940  
 1945  
 1950  
 1955  
 1960  
 1965  
 1970  
 1975  
 1980  
 1985  
 1990  
 1995  
 2000  
 2005  
 2010  
 2015  
 2020  
 2025  
 2030  
 2035  
 2040  
 2045  
 2050  
 2055  
 2060  
 2065  
 2070  
 2075  
 2080  
 2085  
 2090  
 2095  
 2100  
 2105  
 2110  
 2115  
 2120  
 2125  
 2130  
 2135  
 2140  
 2145  
 2150  
 2155  
 2160  
 2165  
 2170  
 2175  
 2180  
 2185  
 2190  
 2195  
 2200  
 2205  
 2210  
 2215  
 2220  
 2225  
 2230  
 2235  
 2240  
 2245  
 2250  
 2255  
 2260  
 2265  
 2270  
 2275  
 2280  
 2285  
 2290  
 2295  
 2300  
 2305  
 2310  
 2315  
 2320  
 2325  
 2330  
 2335  
 2340  
 2345  
 2350  
 2355  
 2360  
 2365  
 2370  
 2375  
 2380  
 2385  
 2390  
 2395  
 2400  
 2405  
 2410  
 2415  
 2420  
 2425  
 2430  
 2435  
 2440  
 2445  
 2450  
 2455  
 2460  
 2465  
 2470  
 2475  
 2480  
 2485  
 2490  
 2495  
 2500  
 2505  
 2510  
 2515  
 2520  
 2525  
 2530  
 2535  
 2540  
 2545  
 2550  
 2555  
 2560  
 2565  
 2570  
 2575  
 2580  
 2585  
 2590  
 2595  
 2600  
 2605  
 2610  
 2615  
 2620  
 2625  
 2630  
 2635  
 2640  
 2645  
 2650  
 2655  
 2660  
 2665  
 2670  
 2675  
 2680  
 2685  
 2690  
 2695  
 2700  
 2705  
 2710  
 2715  
 2720  
 2725  
 2730  
 2735  
 2740  
 2745  
 2750  
 2755  
 2760  
 2765  
 2770  
 2775  
 2780  
 2785  
 2790  
 2795  
 2800  
 2805  
 2810  
 2815  
 2820  
 2825  
 2830  
 2835  
 2840  
 2845  
 2850  
 2855  
 2860  
 2865  
 2870  
 2875  
 2880  
 2885  
 2890  
 2895  
 2900  
 2905  
 2910  
 2915  
 2920  
 2925  
 2930  
 2935  
 2940  
 2945  
 2950  
 2955  
 2960  
 2965  
 2970  
 2975  
 2980  
 2985  
 2990  
 2995  
 3000  
 3005  
 3010  
 3015  
 3020  
 3025  
 3030  
 3035  
 3040  
 3045  
 3050  
 3055  
 3060  
 3065  
 3070  
 3075  
 3080  
 3085  
 3090  
 3095  
 3100  
 3105  
 3110  
 3115  
 3120  
 3125  
 3130  
 3135  
 3140  
 3145  
 3150  
 3155  
 3160  
 3165  
 3170  
 3175  
 3180  
 3185  
 3190  
 3195  
 3200  
 3205  
 3210  
 3215  
 3220  
 3225  
 3230  
 3235  
 3240  
 3245  
 3250  
 3255  
 3260  
 3265  
 3270  
 3275  
 3280  
 3285  
 3290  
 3295  
 3300  
 3305  
 3310  
 3315  
 3320  
 3325  
 3330  
 3335  
 3340  
 3345  
 3350  
 3355  
 3360  
 3365  
 3370  
 3375  
 3380  
 3385  
 3390  
 3395  
 3400  
 3405  
 3410  
 3415  
 3420  
 3425  
 3430  
 3435  
 3440  
 3445  
 3450  
 3455  
 3460  
 3465  
 3470  
 3475  
 3480  
 3485  
 3490  
 3495  
 3500  
 3505  
 3510  
 3515  
 3520  
 3525  
 3530  
 3535  
 3540  
 3545  
 3550  
 3555  
 3560  
 3565  
 3570  
 3575  
 3580  
 3585  
 3590  
 3595  
 3600  
 3605  
 3610  
 3615  
 3620  
 3625  
 3630  
 3635  
 3640  
 3645  
 3650  
 3655  
 3660  
 3665  
 3670  
 3675  
 3680  
 3685  
 3690  
 3695  
 3700  
 3705  
 3710  
 3715  
 3720  
 3725  
 3730  
 3735  
 3740  
 3745  
 3750  
 3755  
 3760  
 3765  
 3770  
 3775  
 3780  
 3785  
 3790  
 3795  
 3800  
 3805  
 3810  
 3815  
 3820  
 3825  
 3830  
 3835  
 3840  
 3845  
 3850  
 3855  
 3860  
 3865  
 3870  
 3875  
 3880  
 3885  
 3890  
 3895  
 3900  
 3905  
 3910  
 3915  
 3920  
 3925  
 3930  
 3935  
 3940  
 3945  
 3950  
 3955  
 3960  
 3965  
 3970  
 3975  
 3980  
 3985  
 3990  
 3995  
 4000  
 4005  
 4010  
 4015  
 4020  
 4025  
 4030  
 4035  
 4040  
 4045  
 4050  
 4055  
 4060  
 4065  
 4070  
 4075  
 4080  
 4085  
 4090  
 4095  
 4100  
 4105  
 4110  
 4115  
 4120  
 4125  
 4130  
 4135  
 4140  
 4145  
 4150  
 4155  
 4160  
 4165  
 4170  
 4175  
 4180  
 4185  
 4190  
 4195  
 4200  
 4205  
 4210  
 4215  
 4220  
 4225  
 4230  
 4235  
 4240  
 4245  
 4250  
 4255  
 4260  
 4265  
 4270  
 4275  
 4280  
 4285  
 4290  
 4295  
 4300  
 4305  
 4310  
 4315  
 4320  
 4325  
 4330  
 4335  
 4340  
 4345  
 4350  
 4355  
 4360  
 4365  
 4370  
 4375  
 4380  
 4385  
 4390  
 4395  
 4400  
 4405  
 4410  
 4415  
 4420  
 4425  
 4430  
 4435  
 4440  
 4445  
 4450  
 4455  
 4460  
 4465  
 4470  
 4475  
 4480  
 4485  
 4490  
 4495  
 4500  
 4505  
 4510  
 4515  
 4520  
 4525  
 4530  
 4535  
 4540  
 4545  
 4550  
 4555  
 4560  
 4565  
 4570  
 4575  
 4580  
 4585  
 4590  
 4595  
 4600  
 4605  
 4610  
 4615  
 4620  
 4625  
 4630  
 4635  
 4640  
 4645  
 4650  
 4655  
 4660  
 4665  
 4670  
 4675  
 4680  
 4685  
 4690  
 4695  
 4700  
 4705  
 4710  
 4715  
 4720  
 4725  
 4730  
 4735  
 4740  
 4745  
 4750  
 4755  
 4760  
 4765  
 4770  
 4775  
 4780  
 4785  
 4790  
 4795  
 4800  
 4805  
 4810  
 4815  
 4820  
 4825  
 4830  
 4835  
 4840  
 4845  
 4850  
 4855  
 4860  
 4865  
 4870  
 4875  
 4880  
 4885  
 4890  
 4895  
 4900  
 4905  
 4910  
 4915  
 4920  
 4925  
 4930  
 4935  
 4940  
 4945  
 4950  
 4955  
 4960  
 4965  
 4970  
 4975  
 4980  
 4985  
 4990  
 4995  
 5000  
 5005  
 5010  
 5015  
 5020  
 5025  
 5030  
 5035  
 5040  
 5045  
 5050  
 5055  
 5060  
 5065  
 5070  
 5075  
 5080  
 5085  
 5090  
 5095  
 5100  
 5105  
 5110  
 5115  
 5120  
 5125  
 5130  
 5135  
 5140  
 5145  
 5150  
 5155  
 5160  
 5165  
 5170  
 5175  
 5180  
 5185  
 5190  
 5195  
 5200  
 5205  
 5210  
 5215  
 5220  
 5225  
 5230  
 5235  
 5240  
 5245  
 5250  
 5255  
 5260  
 5265  
 5270  
 5275  
 5280  
 5285  
 5290  
 5295  
 5300  
 5305  
 5310  
 5315  
 5320  
 5325  
 5330  
 5335  
 5340  
 5345  
 5350  
 5355  
 5360  
 5365  
 5370  
 5375  
 5380  
 5385  
 5390  
 5395  
 5400  
 5405  
 5410  
 5415  
 5420  
 5425  
 5430  
 5435  
 5440  
 5445  
 5450  
 5455  
 5460  
 5465  
 5470  
 5475  
 5480  
 5485  
 5490  
 5495  
 5500  
 5505  
 5510  
 5515  
 5520  
 5525  
 5530  
 5535  
 5540  
 5545  
 5550  
 5555  
 5560  
 5565  
 5570  
 5575  
 5580  
 5585  
 5590  
 5595  
 5600  
 5605  
 5610  
 5615  
 5620  
 5625  
 5630  
 5635  
 5640  
 5645  
 5650  
 5655  
 5660  
 5665  
 5670  
 5675  
 5680  
 5685  
 5690  
 5695  
 5700  
 5705  
 5710  
 5715  
 5720  
 5725  
 5730  
 5735  
 5740  
 5745  
 5750  
 5755  
 5760  
 5765  
 5770  
 5775  
 5780  
 5785  
 5790  
 5795  
 5800  
 5805  
 5810  
 5815  
 5820  
 5825  
 5830  
 5835  
 5840  
 5845  
 5850  
 5855  
 5860  
 5865  
 5870  
 5875  
 5880  
 5885  
 5890  
 5895  
 5900  
 5905  
 5910  
 5915  
 5920  
 5925  
 5930  
 5935  
 5940  
 5945  
 5950  
 5955  
 5960  
 5965  
 5970  
 5975  
 5980  
 5985  
 5990  
 5995  
 6000  
 6005  
 6010  
 6015  
 6020  
 6025  
 6030  
 6035  
 6040  
 6045  
 6050  
 6055  
 6060  
 6065  
 6070  
 6075  
 6080  
 6085  
 6090  
 6095  
 6100  
 6105  
 6110  
 6115  
 6120  
 6125  
 6130  
 6135  
 6140  
 6145  
 6150  
 6155  
 6160  
 6165  
 6170  
 6175  
 6180  
 6185  
 6190  
 6195  
 6200  
 6205  
 6210  
 6215  
 6220  
 6225  
 6230  
 6235